

## UNITED STATES PATENT OFFICE

1,941,204

MANUFACTURE OF USEFUL PRODUCTS  
FROM CELLULOSE DERIVATIVES

Henry Dreyfus, London, England

No Drawing. Application October 18, 1929, Serial  
No. 400,745, and in Great Britain October 29,  
1928

10 Claims. (Cl. 18—54)

This invention relates in particular to the manufacture of filaments, yarns, threads, ribbons or films from cellulose acetate and especially acetone-soluble cellulose acetate.

5 An important object of the invention is to enable an improved drawing out to fine or low filament deniers to be obtained in the spinning of filaments, threads or yarns of or containing cellulose acetate, especially acetone-soluble cellulose acetate.

10 The invention is particularly applicable to the production of filaments, threads, or yarns of low filament denier, from cellulose acetate by evaporative or dry spinning. In the so-called dry spinning or evaporative spinning of filaments, threads or yarns from cellulose acetate solutions, as is known, the solution of cellulose acetate in a solvent or solvent mixture is spun through nozzles or spinnerets into a current or atmosphere of air or other gas, usually of elevated temperature, in spinning cells or chambers, the solvent being thereby evaporated to solidify the filaments.

15 The solvent commonly employed in the spinning solutions is acetone containing a small proportion of water but other volatile solvents or solvent mixtures have also been employed.

20 The discovery has been made that in proportion as one uses increased quantities of water relatively to the solvent, in such spinning solutions, the viscosity of the solution decreases to a lowest figure and then again usually rises with further increase of the amount of water. The curve of viscosity variation of the solutions with 25 the varying amounts of water employed therein, and the point of lowest viscosity attained in the curve are subject to variation according to the characteristics of the cellulose acetate, and, for any given temperature, according to the particular solvent or solvents employed in the solution and the concentration of the solution. It has been found for instance with acetone-soluble cellulose acetate of a character largely employed for spinning yarns, that the viscosity of spinning 30 solutions of for example about 25% concentration prepared by dissolving the acetate in acetone of progressively greater dilution, starting from practically dry acetone, progressively decreases in proportion as the solutions contain 35 more and more water relatively to the acetone, and attains a lowest degree of viscosity at 10-12% of water relatively to 90-88% of acetone after which the viscosity again shows a rise with further increases of water and that the viscosity 40 of the solutions can be reduced to one half or

one third that of the solution in acetone containing very little or no water, by adding relatively substantial quantities of water thereto.

45 The above instance of course is only an illustrative example and in no way limitative, since, as before indicated, the curve drawn to show the relation between the viscosities of the solution and the varying amounts of water employed therein is subject to variation according to a number of factors. It may be mentioned for 50 instance that the point of water dilution of acetone at which the lowest degree of viscosity is attained for a given cellulose acetate varies with the degree or stage to which the given cellulose acetate has been ripened, and in the case of an 55 acetate which has been ripened to a stage of solubility in acetone diluted with considerable quantities of water, the lowest viscosity of solution may, other things being equal, be attained at a higher water content than that indicated in 60 the example above given.

65 It has now been found that the aforesaid solutions of cellulose acetate in acetone containing more than 5 per cent. of water, especially those containing relatively substantial proportions of water, can be readily drawn out into filaments of exceptionally low denier as compared with the filaments obtainable from similar solutions containing no water or comparatively small proportions of water.

70 According to the present invention the production of filaments of low or relatively low denier is carried out by subjecting to a stretch-spinning operation a solution of cellulose acetate in acetone containing more than 5 per cent of water 75 and preferably in acetone containing relatively substantial proportions of water, for example in such proportions as will yield solutions of substantially reduced viscosity as compared with 80 solutions containing small proportions of water 85 or no water. Preferably the water is present in such proportions as to yield cellulose acetate solutions of minimum viscosity or approximately so. In carrying the invention into effect the solutions may, for example, be extruded through suitable 90 orifices into an evaporative atmosphere and the issuing filaments drawn off and wound at such a rate as to stretch and draw them down to the required low denier, e. g. a denier below 3, such as 95 100 105

110 The invention is not restricted to the employment of solutions of any particular lower limit of water content relatively to the acetone, as this may vary as before mentioned, but the proportion of water employed in the solution relatively

- to the acetone will be in general greater than the proportion of about 4.5 to 5 parts by weight of water per 95.5 to 95 parts by weight of acetone, which proportion is usually present in the acetone solutions of cellulose acetate ordinarily employed for spinning cellulose acetate yarns; for example the solutions may contain from about twice this proportion of water and upwards relatively to the acetone, and in particular may contain about 10 to 12 parts of water or more relatively respectively to about 90 to 88 parts or less of acetone, it being understood as before mentioned that the invention is not restricted to these proportions.
- 15 The water will be used in sufficiently large proportion to obtain a solution of the desired viscosity and preferably a solution of or approximately of the lowest viscosity. If lustrous filaments are desired the water should not be added or used in so high a proportion as to cause precipitation of the cellulose acetate under the spinning conditions.

It is understood that the cellulose acetate may be dissolved in the acetone or other solvent or solvents already containing the desired proportion of water or that the required water content of the solutions may be provided for or adjusted by addition of water or further water to previously prepared solutions of the cellulose acetate in the solvent or solvents before or after filtration of the spinning or extrusion solutions.

25 As stated previously filaments of denier below 3, for example 1.5-2.5, may be produced in accordance with the invention, which however is not restricted to these examples as still finer filaments for example of 1 denier or less may be produced.

Again, cellulose acetates of very high or extremely high viscosity characteristics, which property is especially desirable from the point of view of the obtainment of filaments of high quality and strength and regular rounded or bulbous structure, can be employed in the spinning solutions in any desired concentrations whilst permitting the solutions to have a reduced viscosity which allows a greatly improved drawing out of the filaments to low or very low deniers to be secured.

By means of the invention, filaments, yarns or threads can be drawn out to low or very low filament denier, and products of high tensile strength can be produced.

The invention is especially applicable to the production of filaments, threads, yarns, films, and the like from solutions of cellulose acetate in liquids containing acetone as solvent together with the substantial proportions of water, but instead or partly instead of acetone other solvents, whether of higher or lower boiling point, may be used in preparing the solutions, while observing the condition of providing for or adjusting the water content of the solution to the desired reduced viscosity and preferably the lowest degree of viscosity. For example the acetone may contain a small proportion of a solvent of higher boiling point, e. g. diacetone alcohol. The proportion of other solvent may be varied according to its boiling point. If desired, part of the acetone or other solvent or solvent mixture may be replaced by an organic diluent, for example an alcohol, e. g. ethyl alcohol. For instance acetone containing 7-15 per cent of alcohol and 10-5 per cent of water may be used.

The invention applies with particular advantage to the production of filaments, yarns or

threads by evaporative or dry spinning, but it may also be applied to their production by the so-called wet spinning or coagulation method.

Thin or relatively thin ribbons, films, or the like may also be produced in accordance with the invention, the solutions being extruded for this purpose through appropriately shaped dies and formed by evaporation, or run on to forming surfaces or otherwise suitably formed.

80 The invention is specially applicable to the manufacture of filaments, yarns, threads, ribbons and films or the like from cellulose acetate and particularly acetone-soluble cellulose acetate, but it may also be applied, in observing generally similar principles, to the manufacture of yarns, threads, filaments and films or the like from other cellulose esters, for instance cellulose formate, propionate, or butyrate or from alkoxy-alkacyl derivatives of cellulose referred to in the specification of U. S. patent application S. No. 90 348,977 filed 21st March 1929, or "mixed" alkacylalkoxyacyl derivatives of cellulose referred to in the specification of U. S. patent application S. No. 348,978 filed 21st March 1929, or from ethers of cellulose, for instance ethyl, 100 methyl or benzyl cellulose, or the corresponding condensation products of cellulose and glycols or other polyhydric alcohols, or other organic derivatives of cellulose, especially acetone-soluble derivatives.

105 The invention includes not only the process of producing filaments, threads and yarns as herein referred to but also the filaments, yarns and threads produced, and also fabrics made of or containing the same.

110 The invention is illustrated but not limited by the following example.

#### Example

A primary cellulose acetate obtained by 115 acetylating cellulose with acetic anhydride in the presence of acetic acid using sulphuric acid as catalyst, is ripened until it has the desired degree of solubility in acetone containing water, for example in acetone containing more than 10-25 120 per cent of water. There is then prepared a 20-25 per cent solution of the ripened acetate in acetone containing water, the content of the latter being adjusted so that the solution has the desired relatively low viscosity; the water content 125 may be, for example, 10-12 per cent or more e. g. 15-20 per cent. The solution is then spun through suitable orifices into a heated atmosphere, the peripheral speed of the draw-off rollers being adjusted so that the filaments are 130 drawn down to the desired degree of fineness, for example until they are of 1.5-2 denier or less. The filaments so produced may be continuously wound, or twisted and wound, or subjected to other treatments as desired.

135 What I claim and desire to secure by Letters Patent is:—

1. Process for the production of filaments of low denier which comprises spinning and drawing down to filaments of low denier solutions of cellulose acetate in acetone containing sufficient water to yield solutions of substantially lower viscosity than that of solutions of the same concentration in acetone containing 5 per cent of water.

140 2. Process of producing artificial filaments of low denier from cellulose acetate, which comprises spinning a solution of cellulose acetate in acetone containing 10 to 20 per cent of water and 145

- drawing down the filaments until they are of denier below three. 80
3. Process of producing artificial filaments of low denier from cellulose acetate, which comprises spinning a solution of cellulose acetate in acetone containing between 10 and 12 per cent of water and drawing down the filaments until they are of denier below two. 85
4. Process for the production of filaments of low denier which comprises dry-spinning and drawing down to filaments of denier below 3, 90
- 10 solutions of cellulose acetate in acetone containing sufficient water to yield solutions of substantially lower viscosity than that of solutions of the same concentration in acetone containing 5 per cent of water. 95
5. Process for the production of filaments of low denier which comprises dry-spinning and drawing down to filaments of low denier solutions of cellulose acetate in acetone containing 20
- 20 sufficient water to yield solutions of substantially minimum viscosity. 100
6. Process of producing artificial filaments of fine denier from cellulose acetate, which comprises spinning into an evaporative atmosphere a solution of cellulose acetate in acetone containing 10 to 20 per cent of water and drawing down the filaments until they are of denier below three. 105
- 30 7. Process of producing artificial filaments of 110
- 35
- 40
- 45
- 50
- 55
- 60
- 65
- 70
- 75
- low denier from cellulose acetate, which comprises spinning into an evaporative atmosphere a solution of cellulose acetate in acetone containing between 10 and 12 per cent of water and drawing down the filaments until they are of denier below two. 80
8. Process for the production of filaments of low denier which comprises spinning and drawing down to filaments of low denier a solution of an organic derivative of cellulose in acetone containing sufficient water to yield solutions of substantially lower viscosity than that of solutions of the same concentration in acetone containing 5 per cent of water. 85
9. Process for the production of filaments of low denier which comprises spinning and drawing down to filaments of low denier solutions of cellulose acetate in acetone containing an alcohol and also containing sufficient water to yield a solution of substantially minimum viscosity. 90
10. Process of producing artificial filaments of low denier from cellulose acetate, which comprises spinning a solution of cellulose acetate in acetone containing 7-15 per cent of ethyl alcohol and 10-5 per cent of water and drawing down the filaments until they are of denier below three. 100
- HENRY DREYFUS. 115
- 120
- 125
- 130
- 135
- 140
- 145
- 150